

## UNITED STATES PATENT OFFICE

MICHAEL G. CORSON, OF JACKSON HEIGHTS, NEW YORK, ASSIGNEE TO ELECTRO METALLURGICAL COMPANY, A CORPORATION OF WEST VIRGINIA

## ALLOY

No Drawing.

Application filed October 20, 1928. Serial No. 143,017.

This invention relates to an alloy which contains copper as its principal constituent and minor amounts of nickel and beryllium.

A principal object of the invention is to obtain a material having properties which permit of its use for any purpose for which copper is used at the present time and which in addition may have imparted to it by suitable heat treatment hardness and strength far in excess of that possessed by metallic copper.

In my Patent 1,658,186, dated February 7, 1928, I have disclosed that copper and copper alloys containing regulated minor amounts of one or more of certain silicides, among them nickel silicide,  $\text{Ni}_2\text{Si}$ , will assume a remarkably hard and strong condition if subjected to certain heat treatment of the kind to which the term "age-hardening" is usually applied in the art. I have now discovered that a copper alloy containing, in place of nickel silicide, minor amounts of nickel and beryllium may be worked and heat treated in a more or less similar manner.

For example, an alloy containing 95.7% copper, 4% nickel and .3% beryllium can be hot or cold rolled, or otherwise worked, and after the rolling operation subjected to a softening treatment comprising quenching from above 900° C. In this state the alloy is very soft and ductile, and shows a tensile strength of 48,000 pounds per square inch with 60% elongation in two inches. It also possesses a Brinell hardness (500 kg. load, 10 mm. ball) of 52. The quenched alloy can be hardened by subjecting it to a second heat treatment which comprises heating at a temperature within the range of about 350° C. to 700° C. and holding it for a time, depending upon the temperature used and the hardness desired. Heating for a period of approximately 48 hours will secure maximum hardness when a temperature of 350° C. is used, while at a temperature of 700° C. heating for 2 hours will suffice. Alloys of the composition above-mentioned have, when subjected to a hardening heat treatment, attained a Brinell hardness of 110 and a tensile strength of 90,000 pounds per square inch with 15% elongation in two inches. The al-

loy, when in a hardened state produced either by heat treatment or by cold work, shows substantially no diminution in hardness under the influence of heat until a temperature of 700° C. or upwards is reached.

The alloy in the unquenched state is further characterized by the property of self-hardening if air cooled or furnace cooled from 900° C. If cooled in a slow way as compared with air cooling, for instance, when the temperature drops from 900° C. to 700° C. in the course of one and one-half hours, the alloy acquires a hardness of 86 Brinell and a tensile strength of 72,000 pounds per square inch with 25% elongation in two inches.

Copper alloys containing from 0.1% to 2% of beryllium and as high as 40% nickel are considered to be within the scope of the present invention. However, it is preferred that nickel should be present in the proportion of about 13 parts nickel to 1 part beryllium by weight.

The electrical resistivity of the alloys coming within the present invention can be lowered by heat treatment. For example, the alloy of 95.7% copper, 4% nickel and .3% beryllium above-described has an electrical resistivity of 9.3 microhms per centimeter cube when quenched. By subjecting the alloy to a prolonged heat treatment,—i. e., heating at 700° C. for 1 hour and then gradually reducing the temperature over a period of 6 hours to 350° C.—the electrical resistivity of the alloy is brought down to 3.4 microhms or about twice that of metallic copper. A shorter heat treatment,—1 hour at 600° C.—brings the electrical resistivity to 5.2 microhms or about three times that of copper. The unquenched alloy will show approximately the same electrical resistivity if air or furnace cooled from 900° C.

I claim:

- An alloy containing about 0.1 to 2% of beryllium and up to about 40% nickel, with the balance principally copper.
- An alloy containing about 0.3% beryllium and about 4% nickel, with the balance principally copper.
- An alloy containing about 0.1 to 2% of beryllium and about 13 parts nickel to one

part beryllium by weight, with the balance principally copper.

4. An alloy containing about .3 to 2% beryllium, from .1 to 40% nickel and the 5 balance principally copper.

In testimony whereof, I affix my signature.

MICHAEL G. CORSON.

**10**

**15**

**20**

**25**

**30**

**35**

**40**

**45**

**50**

**55**

**60**

**65**